

## UNITED STATES PATENT OFFICE

HELMER BENGSTON, OF INDIANAPOLIS, INDIANA, ASSIGNOR, BY MESNE ASSIGNMENTS, TO ALUMINUM COLORS INCORPORATED, OF INDIANAPOLIS, INDIANA, A CORPORATION OF INDIANA

## PROCESS OF COATING ALUMINUM

No Drawing. Application filed June 23, 1930, Serial No. 463,351. Renewed May 10, 1932.

This invention relates to processes of coating aluminum; and it comprises a method of providing aluminum or aluminum alloys with a decorative, hard, corrosion-resisting 5 coating layer containing  $Al_2O_3$ ,  $SO_3$  and  $H_2O$ , said coating being adapted to be dyed, lacquered and otherwise treated, wherein an article of aluminum or aluminum alloy is temporarily made an anode in rather strong 10 sulfuric acid, the specific gravity being between 1.5 to 1.7 and the acid advantageously containing a considerable proportion of glycerin or another inhibitor, all as more fully hereinafter set forth and as claimed.

15 As is well known, ordinary aluminum articles are covered with a hard coherent coating of aluminum oxid formed by the action of air. This coating is self-renewing in the sense that where it is removed, cracked or 20 broken it is, practically at once, renewed by the action of the air. While this coating is excellent protection against corrosion and is not unsightly, its existence precludes the ordinary decorative treatments which can be 25 applied to other metals. It is, for example, difficult to make different finishes by different ways of buffing or polishing; and the coating does not give good anchorage to lacquers and varnishes. For this reason, aluminum articles are seldom decorated in any way. 30 Plating is difficult.

It is an object of this invention to obviate difficulties in decorating articles made of aluminum and aluminum alloys by substituting 35 for the ordinary oxid film a special coating produced by anodic treatment of the aluminum in a special way. It has been found that if an article of aluminum, or of aluminum alloy, is thoroughly cleaned and 40 buffed and is then made an anode in strong sulfuric acid of 1.5 to 1.7 specific gravity there develops a hard coating of substantial thickness. The coating is insoluble in water, contains sulfuric acid in combination with 45 the alumina in an insoluble form and has an empirical composition corresponding to that of a highly basic hydrated sulfate of alumina. It is minutely pervious but the porosity is sub-microscopic in character and the pores 50 are readily sealed to give a completely pro-

tective weather-proof layer. This coating is colorless but, as I have found, the contained material is in such a reactive form as to take up and readily hold those dyes which are customarily used with mordants. In 55 other words, the alumina compound can be converted into a "lake" of any desired color or hue.

Decorative on the coating produced as described may be achieved in a number of other ways. Its thickness is sufficient to permit 60 buffing and mechanical finishing. And it is found that in spite of the minute character of the pores, it will readily take up oils and oily materials. This ready permeability by oils 65 is possibly connected with the adsorbent nature of the material of the coating; a view which is supported by the fact that oils once taken up are removed with difficulty by gasoline and other oil solvents. Colored oils 70 give various decorative effects.

The strength of the sulfuric acid used in the electrolytic treatment is of great importance. The best results are given by a sulfuric acid of a specific gravity of 1.5 to 1.7; 75 that is an acid containing from 60 to 77 per cent of  $H_2SO_4$ . A 64-65 per cent acid is generally useful. Solutions somewhat stronger and weaker than those in this range will operate for my purposes but are open 80 to objection. With higher specific gravities, the conductivity is lessened to an extent making it difficult to secure efficient current densities while certain lower specific gravities, those between 35 and 60 per cent acid, give 85 too much conductivity and also cause excessive etching and attack on the aluminum. No etching or attack on the aluminum surface is here desired other than that necessary in forming the coating. It has been found 90 highly advantageous, even in using the optimum concentration of sulfuric acid, to add some glycerin to the solution. This decreases etching and attack still further. I use ordinarily about 1 part by volume of 95 glycerin to 15 parts by volume of the 1.5-1.7 acid. In the presence of the glycerin the specific gravity can be lowered a little below the range mentioned without too much attack and with the possibility of using higher 100

current densities. Other inhibitors may be used in lieu of glycerin for diminishing solution of metal or coating. The aluminum sulfate in solution is an inhibitor and it is often worth while to saturate the acid initially with aluminum sulfate.

Other acids, such as nitric acid, are not here the equivalent of sulfuric acid since they cause surface roughening and attack 10 without production of the type of coating here desired. The sulfuric acid should be free of HCl or chlorids, as these cause too much solution loss.

In operation, the apparatus in which the 15 anodic coating is effected is most conveniently made of stoneware or other ceramic or vitreous material. However, containers of wood or metal, lined with materials resistant to sulfuric acid, such as pitch, rubber or 20 sheet lead, may be used. The cathodes may be of any convenient material, but I find cathodes of ordinary chemical lead best adapted. The size and shape of the cathodes, of course, vary according to the work 25 to be done; but for many purposes they may be located on the side walls of the bath and cover about 50 per cent of the side wall area. With lead lined containers the lead lining may very conveniently serve as a cathode. 30 The articles to be treated may be hung in the bath upon the usual conducting rods. Pointed clamps may be used with sufficient passage of current so that the uncoated area in the finished article is merely an imperceptible 35 spot. The direct current voltage used is ordinarily about 12 volts between terminals. With a voltage of this order no rheostats or regulating devices are necessary. The bath is cooled in any of the ordinary ways. 40 With large baths, cooling coils or cooling jackets are generally desirable. Circulation of the electrolyte, with agitation thereof, in well known ways, is also desirable. Heat is evolved in the operations. It is best to keep 45 the temperature between 20° to 30°, preferably at 25° C. The anode current density, with the usual spacing between anodes and cathodes, is ordinarily between 6 and 10 amperes per square foot of surface of the article being treated.

The aluminum articles to be coated should be subjected to the usual preliminary cleaning treatments. Where a lustrous coating is wanted the aluminum should be buffed before dipping. In any event, grease and other foreign matter should be removed.

For most purposes the time required for the anodic treatment to produce the desired coating is 10 to 30 minutes. However, a useful layer may be formed in 5 minutes or less and of course an extended time of an hour or more does no harm. Flow of current decreases with the increase in thickness of the coating and after a normal coating has been formed, prolongation of treatment effects no

material change. Coating is uniform at all points in free contact with the bath whatever the contour of the article, the increase in current at any thin spot effecting this evenness automatically.

Agitation is desirable during the coating operation for various reasons including that of avoiding formation of gas pockets in reentrant portions.

With any strength of acid within the range given, there is but little useless attack on the metal or the coating by the formation of dissolved sulfate of alumina and this can be further reduced by the use of inhibitors. For the most part, the aluminum oxidized in the anodic treatment reappears in the coating. Such aluminum as does dissolve forms aluminum sulfate which after a time crystallizes out.

If the work is not completely clean there is apt to be uneven coloring due to varying thicknesses of coating. In such an event, it is best to remove the coating and reprocess the article. For removing the coating a 5 to 10 per cent hydrofluoric acid dip is most satisfactory. On immersion the coating rapidly dissolves, solution taking perhaps 15 seconds. There is then a vigorous evolution of gas as the acid reaches the metal. When this occurs, the metal is removed, washed and is ready for processing.

After treatment the article is removed, rinsed and dried. The coating is insoluble in water at the ordinary temperature and is not injured by rinsing. Thorough rinsing to remove contained electrolyte is desirable. The wet coating after rinsing may be dyed by treatment with a solution of a dye; the dye being taken up to form what may be termed a "lake". The dye is found to penetrate the coating and give uniformity of color at all points. Exhaustion of the dye bath is usually good. The coating may be buffed and mechanically finished, before or after the application of dye. Alternatively, in lieu of dyeing the coating it may be oiled with a suitable oil such as lanolin or lard oil. Neutral petroleum oils and waxes may also be used. Apparently the oil is taken up in the body of the coating and not merely superficially. In buffing, the coating usually takes up oily matter from the buffing compound. The dyed coating is usually dried and buffed or otherwise finished. It may be oiled.

The anodic treatment described usually gives a coating of about 0.0005 inch thick. With a somewhat greater time of anodic treatment the thickness of coating may be 0.0015 inch or more. These thicknesses are sufficient for all ordinary purposes, and while somewhat thicker coatings may be secured the result is more attack on the underlying aluminum.

The coating thickness varies directly with the potential of the bath and, for a time, with

sulfuric acid diluted to 1.5 to 1.7 specific gravity.

5. In electro-coating articles of aluminum and aluminum alloys, the process which comprises making such an article an anode in sulfuric acid diluted to 1.5 to 1.7 specific gravity, such acid containing a little glycerin.

6. In electro-coating articles of aluminum and aluminum alloys, the process which comprises passing current between such an article and another electrode in an electrolytic bath of sulfuric acid diluted to 1.5 to 1.7 specific gravity.

7. In electro-coating articles of aluminum and aluminum alloys, the process which comprises anodically coating the said articles in a bath of sulfuric acid diluted to 1.5 to 1.7 specific gravity, rinsing, and dyeing the said coating.

20 8. In electro-coating articles of aluminum and aluminum alloys, the process which comprises anodically coating the said articles in a bath of sulfuric acid diluted to 1.5 to 1.7 specific gravity, rinsing the coating and plugging the pores thereof, whereby the article becomes resistant to corrosion.

30 9. In electro-coating articles of aluminum and aluminum alloys, the process which comprises anodically coating the said articles in a bath of sulfuric acid diluted to 1.5 to 1.7 specific gravity, rinsing the coating, plugging the pores thereof and finally buffing the said coating.

35 10. In electro-coating articles of aluminum and aluminum alloys, the process which comprises anodically coating the said articles in a bath of sulfuric acid diluted to 1.5 to 1.7 specific gravity and thereafter mechanically finishing the article.

40 40 In testimony whereof, I have hereunto affixed my signature.

HELMER BENGSTON.

the duration of treatment. Thickness varies somewhat with the strength of acid. In the process as described the coatings produced have a thickness of the order of thousandths of an inch.

6 In coating, some of the metal goes into solution in the acid as aluminum sulfate and after a time the acid becomes saturated and deposits crystals. To dispose of this crystallized sulfate and keep down the temperature of the bath, it is usually expedient to keep a portion of the bath in cyclic circulation to and through a filter and cooling means and back to the bath. A leadlined pump may 10 be used.

15 While I have described making the aluminum an anode in a sulfuric acid bath with employment of direct current of the usual type used in plating, an alternating current 20 may be used in lieu of direct current. The "rectifier" action of aluminum makes this feasible. I have secured good coatings with low voltage alternating current. Even 8 volts have sufficed. In some instances this applicability of alternating current is advantageous since a small step-down transformer can be used in lieu of the more complex equipment necessary in securing low voltage direct current from ordinary 60 cycle 25 110 volt alternating current.

30 Some properties of a coating produced by the anodic treatment are as follows: it is a non-conductor of electricity when dry and particularly when oiled, evincing a good resistance against spark puncture; it is readily reactive with, adsorbs and permanently holds organic dyes; it is resistant to water and wear; it stands buffing and takes a high polish; it withstands heating without lifting or 35 breaking away from the metal; it withstands punching, stamping and the like to a reasonable degree; it binds paints, oils, enamels, lacquers and the like; it shows no definite crystalline structure under X-ray examination; and it is a coating of reasonable thickness rather than a film. While the coating 40 is, as stated, amorphous or non-crystalline under the X-ray, it has a laminar structure. Next to the metal is an extremely thin, extremely hard, glaze-like layer while there is a 45 much thicker outer layer of considerably less hardness integrally attached thereto. The hardness of this outer layer however is sufficient to permit buffing and polishing etc., as stated. The sub-microscopic porosity extends 50 through both layers and is of a type like that with "silica gels", the amount of internal surface being very great. This, together with the transparent nature of the coating, is an 55 explanation of the bright and true colors which can be obtained in dyeing. In one particular coating about 0.00066 inch thick, the porosity represented about 40 per cent of the 60 total film. The coating is resistant to heat, 65 withstanding temperatures up to, say, 300° C.,

without shelling or cracking and without much loss of water. With well rinsed material, the amount of hygroscopic moisture given up at 100° C., is very little. The rest of the H<sub>2</sub>O is more permanently held. The 70 coating is tolerably resistant to acids but loses sulfuric acid in alkaline liquids. It is insoluble in cold water but gives up sulfate to boiling water. Two hours boiling with distilled water are however required for completion of the action. Rinsed, dry material does not corrode in the air and with the pores plugged or filled, corrosion by sea water does not occur. As illustrating the adsorptive 75 power of the coating material, it may be mentioned that on application of lacquers containing dyes, some of the dye sometimes migrates into the underlying coating.

80 Aside from its advantageous mechanical properties, the present coating owes most of its value to its highly developed adsorptive power; a power which enables it to take up and hold oils, coloring matters, etc. against withdrawal. I attribute this high adsorptive power in part to the large amount of fixedly 85 contained SO<sub>3</sub> or basic aluminum sulfate as the case may be. This basic sulfate is in a form resisting action by cold water and it is extremely active as an adsorbent. In the 90 article of the present invention, the fixedly held SO<sub>3</sub> may range between, say, 16 percent and 23-24 per cent of the coating. Using weaker sulfuric acid than 1.5-1.7 specific gravity, it is not possible to fix as much SO<sub>3</sub> and the adsorptive properties are not as good. 95

100 The present application contains certain matter in common with prior and copending application 368,742 filed June 5, 1929, and is filed as a substitute for and continuation in part of said application. Aluminum coated with the described coating produced by the present process is not specifically claimed herein, it forming the subject matter of another and copending application, Serial No. 460,543, filed June 11, 1930.

110 What I claim is:

1. In electro-coating articles of aluminum and aluminum alloys, the process which comprises making such an article an anode in sulfuric acid diluted to about 64-65 per cent 115 H<sub>2</sub>SO<sub>4</sub>.

2. In electro-coating articles of aluminum and aluminum alloys, the process which comprises making such an article an anode in sulfuric acid diluted to about 64-65 per cent 120 H<sub>2</sub>SO<sub>4</sub> and containing a little glycerin.

3. In electro-coating articles of aluminum and aluminum alloys, the process which comprises making such an article an anode in sulfuric acid diluted to about 64-65 per cent 125 H<sub>2</sub>SO<sub>4</sub> and containing an inhibitor.

4. In electro-coating articles of aluminum and aluminum alloys, the process which comprises making such an article an anode in 130